

May 8, 1934.

W. D. HODSON ET AL.

1,957,456

METHOD OF AND APPARATUS FOR TREATING METAL CASTINGS

Filed Jan. 27, 1930



FIG. 4



FIG. 1

FIG. 2

Inventors:  
Walter D. Hodson <sup>and</sup>  
Ira J. Simmmons  
By Dryenforth, Lee, Britton and Miles  
Atty's.

## UNITED STATES PATENT OFFICE

1,957,456

METHOD OF AND APPARATUS FOR TREAT-  
ING METAL CASTINGSWalter D. Hodson, Chicago, Ill., and Ira J.  
Simmons, Clairton, Pa.

Application January 27, 1930, Serial No. 423,811

5 Claims. (Cl. 148—2)

The invention relates to a method of, and apparatus for treating metal castings, and more particularly to a method of, and apparatus for retaining the heat in and equalizing the temperature in steel ingots or castings after the pouring operation.

The improved method is preferably practiced by removing the mold from an ingot or casting, after the pouring operation, substantially as soon as it has cooled sufficiently to become self-supporting and then promptly placing a thermally insulating housing or hood over the ingot or casting to retain the heat therein and to retard the cooling thereof so that relatively equal temperatures will prevail throughout the ingot or casting after it has been left to soak in its own sensible heat for some time. This treatment reduces the amount of pipe that will form, and also prevents the formation of the relatively large amount of surface cracks, oxide, and other flaws or undesirable characteristics that result from practicing the methods now widely used.

The method is preferably practiced with apparatus comprising a thermally insulating housing or hood, the hood being preferably of such size that there are dead-air spaces between the ingot and the inner surfaces of the hood. The invention permits one to equalize the temperature of the ingot without placing it in a heated soaking pit before the rolling operation, as is the practice usually followed. This effects a saving of labor and fuel, and has many other advantages hereinafter set forth.

In the drawing, wherein we have illustrated apparatus embodying a preferred form of the invention:

Figure 1 is a vertical section through a car supporting a mold in which an ingot has been poured.

Fig. 2 is a central section taken through the apparatus shown in Fig. 1, the mold having been replaced by a thermally insulating housing, or hood.

Fig. 3 is a section taken on line 3—3 of Fig. 2, and

Fig. 4 is an enlarged section taken on line 4—4 of Fig. 2.

At the present time it is common practice in connection with open hearth steel to pour the metal into ingot molds which are mounted on cars carried past the ladle, the molds being removably mounted on a part of the car which is called the "stool". As soon as the ingot has cooled sufficiently to be handled the mold is removed and the ingot is picked up and placed in a heated soaking pit where it is equalized.

In practicing our improved invention in connection with the production of steel, we preferably make use of the cars which carry the molds past the ladle, but our invention is limited to the use of cars and to the manufacture of steel only to the extent indicated in the appended claims, as the invention may be practiced in connection with other metals.

In Figs. 1 and 2, we have shown cars 4 provided with suitable wheels and adapted to carry stools 3 and molds 1 past the ladle. The cars 4 are preferably provided with apertured platforms 4a, the apertures being adapted to receive lugs 3a formed upon the stools 3. The stools 3 are preferably formed from metal and are preferably provided with upwardly extending flanges 3b and 3c, the flanges 3c being adapted to hold mold 1 in place upon the stool. It will be noted that the mold 1 rests upon a thermally insulating pad 2 which is preferably formed from refractory cementitious material, or the equivalent. This pad prevents rapid cooling of the bottom of the ingot. The flanges 3b are adapted to hold a thermally insulating hood 5 in place upon the stool when the mold 1 has been removed from the ingot cast within the mold. In the drawing, the ingot is identified by the reference character 9.

The hood 5 preferably comprises an outer shell or housing 7 which is preferably formed from cast iron, or the equivalent for the purpose, and is preferably provided with lugs 5a to facilitate the handling thereof. A lining 6 of refractory cementitious material, or the equivalent, is preferably provided within the housing 7 and is preferably held in place within the housing by inwardly extending flanges 7a provided in the base of the housing. As best shown in Figs. 2, 3 and 4, the outer surface of the lining 6 is preferably corrugated to provide a plurality of dead-air spaces 6a between the lining and the housing.

The hood 5 is preferably of such dimensions that a dead-air space 8 is provided around the sides and top of the ingot 9 when the hood is placed upon the stool in a manner illustrated in Fig. 2.

In practicing the improved method, we preferably mount a plurality of molds 1 on a like number of cars 4, in the manner illustrated in Fig. 1, and the cars are moved past the ladle, each load receiving the usual charge of fused metal to form an ingot of the desired dimensions. When the ingots have become self-sustaining, we remove the molds 1 therefrom and place the hoods 5 on the stools 3 in the manner indicated in Fig. 2 so that the ingots are thermally insulated by the dead-air spaces 8 as well as by the walls of the

hoods 5. Therefore, the sensible heat of the ingots is largely retained within the hoods 5 and the temperatures thereof are equalized by making use of this heat. We find that as soon as the 5 hoods are placed over the ingots contraction of the surfaces ceases for a relatively long period of time as the inner or central parts of the ingots are relatively hot as compared with the outer surfaces thereof and the placing of the hoods 10 over the ingots retards the loss of heat from the surfaces of the ingots to such an extent that they will heat to higher temperatures by heat conducted from the interiors of the ingots. This method of equalizing the temperatures thereof 15 is exceedingly advantageous when compared with the usual practice of normalizing in heated soaking pits. Thus, when the ingots are to be reheated and the temperatures thereof equalized in a soaking pit they are subjected to the atmosphere before and after they have been placed 20 in the pits. This results in the formation of oxide in relatively large quantities as compared to that which forms upon and in ingots which have their temperatures equalized in accordance 25 with our improved method, it being readily understood that when our improved method is practiced the ingots are exposed to the atmosphere for an exceedingly short time and the amount of air with which they come in contact 30 is afterwards limited to that in the dead-air spaces 8.

When the temperature of ingots are equalized by the soaking pit method, they contract a relatively large amount before they are placed in 35 the pit, and therefore a relatively large amount of gas is occluded from them. Then when the ingots expand in the heated pit they absorb much gas which results in oxidation within the ingots and also results in innumerable small gas filled 40 pockets or holes. These conditions do not obtain when the temperatures of the ingots are equalized by retaining the sensible heat thereof during the temperature equalizing process so that it is unnecessary to reheat them:

45 Another advantage of our improved method is that comparatively few surface cracks form in the ingots, and these cracks do not penetrate to any great depth. Obviously, such cracks are not as numerous and deep in a finished bar formed 50 from an ingot subjected to our improved method as there are in a bar formed from an ingot subjected to the soaking pit method. Still another and exceedingly important advantage of our improved method is that relatively little pipe forms 55 in ingots produced by practicing our method as the ingots need not be cooled to a temperature which permits handling thereof as is the practice in the heated soaking pit method. The savings effected through the reduction of pipe when 60 our method is practiced are considerable as our method in itself does not necessitate employing other expedients to reduce the formation of pipe.

Our method is preferably practiced so that the ingots are rolled when they have been cooled to the proper rolling temperature. This practice also effects savings in that it is unnecessary to place the ingots in a soaking pit to reheat them. If the ingots are not to be rolled promptly the hoods are preferably left in place upon the stools until the temperature of the ingots is low enough so that they can be exposed freely to the atmosphere without causing the formation of any appreciable amount of oxide.

80 We have found that when our method is practiced, it results in a relatively better rolling steel due to the thoroughness with which the temperature thereof is equalized. We have also noted 85 that there is a reduction in the usual loss due to burned steel.

90 While we have shown and described certain embodiments of our invention, it is to be understood that it is capable of many modifications. Changes, therefore, in the construction and arrangement may be made without departing from the spirit and scope of the invention as disclosed 95 in the appended claims, in which it is our intention to claim all novelty inherent in our invention as broadly as possible, in view of the prior art.

100 What we regard as new, and desire to secure by Letters Patent, is:

1. A method of preparing an ingot for rolling 105 which comprises covering said ingot with an insulating hood substantially as soon as it becomes self sustaining after the pouring operation, and then soaking said ingot solely in its own heat until it cools to an equalized temperature sufficiently low for the rolling operation.

110 2. The method of equalizing the temperature of a metallic ingot having an initial average temperature above a rolling temperature which comprises covering said ingot with an insulating hood 115 of dimensions of the same order as the ingot and having negligible heat capacity, and maintaining said ingot therein until its temperature is substantially equalized throughout and said ingot has reached a rolling temperature.

120 3. The method of preparing a metallic ingot for rolling which comprises pouring molten metal into a mold, cooling the metal to a condition of external rigidity and removing the molds and immediately covering the ingot with an insulating substantially airtight hood, maintaining the ingot beneath said hood until the temperature of the ingot is substantially equalized throughout and said ingot has cooled to a rolling temperature.

125 4. The method as set forth in claim 3, in which said hood has a negligible heat capacity.

130 5. The method as set forth in claim 3, in which the ingot is not removed from its initial base throughout the operation.

135 WALTER D. HODSON.  
IRA J. SIMMONS.